

## UNITED STATES PATENT OFFICE

HENRY PHILIP SHOPNECK, OF DORCHESTER, MASSACHUSETTS, ASSIGNEE, BY MESNE ASSIGNMENTS, TO ARDEN BOX TOE COMPANY, OF WATERTOWN, MASSACHUSETTS, A CORPORATION OF MASSACHUSETTS

## WATER-LAID FELT, WOOL FIBER

No Drawing.

Application filed June 29, 1926. Serial No. 119,479.

In my prior Patent, No. 1,574,126, granted February 23, 1926, I disclosed a water-laid felt consisting of a short-fibered base, such as wood pulp, and relatively longer vegetable fibers of ligno-cellulosic origin distributed throughout the base in felted relation therewith.

I have now discovered that I may substitute for the long vegetable fibers of my 10 said prior patent certain other long fibers not of ligno-cellulosic origin, such as wool fibers, or a mixture of wool and cotton fibers. These fibers are obtained from usual sources. Preferably, I use long fibered shredded textile rags, clippings, or new cuttings. By 15 the term "textile rags" I mean cotton rags containing more or less wool, and wool rags substantially free from or containing only a small percentage of cotton.

20 The long wool or wool and cotton fibers are mixed with the short fibered base and the mass is felted out, preferably on a cylinder felting machine, and afterwards impregnated with a binder, as a thermo-plastic binder, 25 a characteristic mix consisting of approximately 60% short fibered stock, and 40% long fibers of the class described.

Under some circumstances, I may use mineral fibers (such as asbestos), a characteristic 30 mix consisting of approximately 60% short fibered stock, 30% long fibers of the class described, and 10% asbestos or other mineral fibers. The asbestos fiber, being non-combustible, diminishes the combustibility of the 35 finished product, while at the same time serves as the short-fibered or long-fibered component, depending upon the kind of asbestos fiber used.

It is to be noted that in the two examples 40 given the felt consists of a preponderant proportion of short-fibered stock and a subordinate proportion of long-fibered stock. When these stocks are used in substantial proportions in the examples, namely 60% 45 short-fibered stock and 40% long-fibered stock, it is possible to produce a product which is well felted and of uniform texture, owing to its content of short fibers, and at the same time possess high absorbency and 50 tear resistance, owing to its content of long

fibers. Such a product is an excellent base or foundation material for impregnation with thermo-plastic binder in the production of box toe material which is capable of being softened by heat to permit a box toe blank cut therefrom to conform to the shape of the last, as hereinafter claimed. 55

Various other modifications in materials and proportions may obviously be resorted to all without departing from the spirit of 60 my invention, if within the limits of the appended claims.

What I therefore claim and desire to secure by Letters Patent is:

1. A water-laid felt consisting only of a 65 short fibered base and much longer wool and cotton fibers and asbestos fibers distributed therethrough in felted relation therewith, the proportions of the mix being substantially as follows: short fibered base 60%, wool and cotton fibers 30% and asbestos fibers 10%. 70

2. A water-laid felt consisting of a short-fibered base and much longer wool and cotton fibers and asbestos fibers distributed therethrough in felted relation therewith. 75

In testimony whereof I affix my signature. 80  
HENRY PHILIP SHOPNECK.

80

85

90

95

100